

May 7, 1935.

A. M. GRONNINGSAETER

2,000,171

REDUCTION OF OXYGENEOUS NICKEL OR NICKEL COPPER COMPOUNDS

Filed Aug. 15, 1933

2 Sheets-Sheet 1



May 7, 1935.

A. M. GRONNINGSAETER

2,000,171

REDUCTION OF OXYGENEUS NICKEL OR NICKEL COPPER COMPOUNDS

Filed Aug. 15, 1933

2 Sheets-Sheet 2

Fig. 2.



Fig. 3.



Fig. 4.



INVENTOR

Anton Martin Gronningsaeter

BY

Parsons, Darvin, Mason & Edmonds

ATTORNEY

## UNITED STATES PATENT OFFICE

2,000,171

REDUCTION OF OXYGENEOUS NICKEL OR  
NICKEL COPPER COMPOUNDSAnton Martin Gronningsaeter, New York, N. Y.,  
assignor to Falconbridge Nickel Mines Limited,  
Toronto, Ontario, CanadaApplication August 15, 1933, Serial No. 685,225  
In Norway August 27, 1932

2 Claims. (Cl. 75—66)

This invention relates to the reduction of oxygenous nickel or nickel-copper compounds by means of gaseous reducing agents and more particularly to the reduction of materials obtained by roasting sometimes followed by leaching of nickel copper matte.

It is known that nickel oxide is reduced by watergas at a temperature of 350°—400° C. and higher. This reaction is made use of for example in the manufacture of nickel for use as a catalyst and in the Mond process for the refining of nickel.

In the Mond process the reduction is carried out in multiple hearth furnaces of iron with a revolving shaft carrying arms with rabbles, by means of which the material is stirred and moved from hearth to hearth. To maintain the reaction temperature, outside heat must be supplied. For this purpose some of the floors of the furnace are provided with interior chambers (muffles) through which hot gas is passed. It is self-evident that the temperature of the muffle floors must be higher than that desired in the treated material. This fact, however, represents a factor of risk because the reduced nickel has a tendency to sinter by being brought into immediate contact with the hot muffle floor, so that it "cakes" and becomes hard.

The difficulties become particularly great when for some reason it is desired to effect the reduction at a comparatively high temperature near the sintering temperature of the reduced nickel material. This is for example the case in the manufacture of nickel material to be employed for cementing out copper, for neutralizing acidic nickel salt solutions and for the like purposes.

Other inventors have proposed for the purpose of extraction of nickel, to reduce nickeliferous ores by heating with reducing gases having a temperature higher than that which is needed for reduction of the nickel. In these cases however, no particular attention is paid to the physical and chemical properties of the product obtained, which in these cases are of no great importance. The reactivity of the reduced nickel obtained is greatly dependent on the temperature during the reduction. If the temperature rises too high, sintering will occur, and this will unfavourably affect the reactivity of the product obtained, and may at the same time cause considerable mechanical troubles with the operation of the furnace; sintering in the present case will therefore cause great prac-

tical drawbacks in the preparation and the use of the product.

The present invention has for its object a process by means of which it is made possible to effect the reduction at such elevated temperatures as mentioned above—for example between 400 and 550° C. without the above mentioned drawbacks of sintering and caking of the reduced material making itself felt.

It is characteristic for this process that the heating does not or only in part take place indirectly through the muffle walls; the heating, at least partly, takes place directly by effecting the reduction by means of a reducing gas having, when it enters the furnace, a temperature which is considerably higher than that at which the reduction takes place. If the reduction is to be effected at a temperature of 400—550° C. it will for example be suitable to use a reducing gas having a temperature of between 500° and 700° C. at the point of entrance into the furnace. The heat content of the gas will then, as experience has proved, usually be sufficient to heat the furnace and the material to the desired temperature. The temperature of the entering reducing gas is so controlled as to maintain the material leaving the reduction space at a temperature of between 400—550 degrees centigrade.

When the furnace is operated in this way, the floor on which the material rests and against which it is pressed by means of the rabbles, will have a lower temperature than the material itself so that local overheating will not take place.

The supply of heat to the furnace may in its entirety be effected by means of hot reducing gas but this method may also be combined with the above mentioned indirect heating, for example by passing gases having approximately the same temperature as that at which the reduction shall take place, through the muffle floors of the furnace. It is usually preferred, however, to limit the use of indirect heating to the upper floors, where the material is dried and preheated.

When the furnace is operated in accordance with the invention, it has been found to be possible to maintain the material in the critical zone of the furnace at a temperature just below the sintering temperature of the reduced material—for example of about 450—500° C. or even higher—without meeting any drawbacks in the form of sintering or "caking." By these means

increased capacity of the furnace and a better utilization of the reducing gases are obtained at the same time as it is made possible to operate the furnace uninterruptedly for very long periods of time without mechanical difficulties of any kind. Direct heating by means of the reducing gas in the present instance results in economical advantages of great importance.

The furnace should be insulated against heat losses by radiation and convection for example by lining with asbestos, insulating bricks and the like. This brings about reduction of heat losses and also a more uniform distribution of the heat and a more uniform temperature throughout the whole body of treated material, which also counteracts local overheating.

The heating of the reduction gas may take place in several different ways. A particularly advantageous way of heating consists in producing the required gas in an electrically heated watergas generator, from which the gas escapes at a temperature suitable for introduction into the reduction furnace. If it is found that the gas coming from the gas generator in some instance has too low a temperature for the purpose, the gas on its way to the reduction furnace may be passed through a heating apparatus of a suitable construction, for example an electric furnace. The invention may be considered in conjunction with the following description and the accompanying drawings, in which:

Fig. 1 is an elevation partly in section of a reduction furnace of the character above mentioned;

35 Fig. 2 is a section on the line 2—2 of Fig. 1;  
Fig. 3 is a section on the line 3—3 of Fig. 1; and

40 Fig. 4 is a section on the line 4—4 of Fig. 1.  
The reduction furnace shown is of the multiple hearth type, comprising a plurality of spaced and superposed shelves 10 laterally supported in close proximity to a shaft 11 centrally and vertically disposed within a heat-insulated outer furnace shell 12. The shaft is appropriately supported on its bottom, and is provided with suitable driving gears. A plurality of spaced and superposed muffles 13 alternate with the shelves, the tops of the muffles being adapted to function as shelves. An annular space 14 is provided between the central shaft and the muffles. Each muffle (see Fig. 3) has a damped gas inlet 15, and a gas outlet 16.

45 A feed hopper 17 is mounted on the top of the furnace structure, the lower end of the hopper being provided with a damper to regulate the amount of finely divided material deposited onto the top shelf of the furnace. The central shaft is provided with a series of spaced and superposed rabble arms 18 provided with teeth 19 adapted to scrape against the tops of the muffles and shelves. The bottom of the furnace is provided with an outlet 20, which communicates with a hopper 21 for receiving finely divided nickel powder.

50 Referring to Fig. 1, a water gas generator 22 communicates by means of a conduit 23 with a gas preheater 24. The preheater in turn communicates with the bottom of the reduction furnace by means of a conduit 25. Spaces 26 are provided between the shelves and the central shaft to permit the upward passage therethrough of gases and the downward passage therethrough of rabbled material. A gas offtake 27 communicates with the top of the reduction

furnace and extends to the bottom of a combustion chamber 28 communicating with a gas distributing chamber 29.

55 Referring to Figs. 2 and 3 more particularly, it will be seen that the distributing chamber 29 is separated by a wall from a spent gas receiving chamber 30 that communicates with a stack 31.

In operation, finely divided leached matte, consisting, for example, of a mixture of nickel oxide (60-65% nickel) and copper oxide (11-14% copper) is introduced into feed hopper 17, from which regulated amounts are intermittently dropped onto the top muffle 13 by suitable operation of the hopper damper. The central shaft 11 is set in motion, which operates to rotate rabble arms 18 and their scraping teeth 19.

At the same time, reducing gas produced in generator 22 is introduced into the bottom of the reduction furnace by way of inlet 25. This gas may or may not be preheated in the preheater 24, as desired or necessary to accomplish the desired type of reaction within the reduction furnace. The gas is preferably made to enter the bottom of the reduction furnace at a temperature of 500-700° C. The gas rises upwardly through passageways 14 and 26, while rabbled matte material falls downwardly through the same passageways. It will thus be seen that the matte in finely divided form is progressively advanced through the reduction zone of the furnace in a direction generally counter-current to and in direct contact with the hot reducing gases, which are at a temperature sufficiently high to effect reduction of oxygeneous nickel compounds present in the matte. At the same time, the temperature of the gases is carefully selected so that the matte material does not fuse. In this manner, a highly reactive nickel powder is obtained.

40 In a present preferred practice of the invention, the finely divided matte material is also indirectly heated. To this end, the gases leaving the top of the furnace by way of outlet 27 are passed into the combustion chamber 28 where they are ignited. The hot gaseous products of combustion then pass into the distributing chamber 29 where they may be by-passed through one or more of the muffles 13. Gas thus entered into a muffle by way of inlet 15 passes completely through the muffle and out at the exit 16 into the spent gas receiving conduit 30, from which it escapes through the stack 31. The amount of gas introduced into the muffle is properly regulated by operating the dampers 16.

45 Since the gases produced in generator 22 are introduced into the bottom of the reduction furnace at substantially their maximum temperature, it may usually not be advisable to effect maximum simultaneous indirect heating of the matte material undergoing rabbling. Under this circumstance, it is advisable, for example, to close the dampers of the lowermost muffles, and then only pass gaseous products of combustion through one or more of the uppermost muffles.

50 As stated above, in the present preferred practice of the invention, hot reducing gases are introduced into the bottom of the reduction furnace at a temperature of 500-700° C. The material withdrawn from the bottom of the reduction furnace has a temperature of 450-500° C. or even higher.

55 By following the procedure herein outlined, the reactivity of the nickel powder produced is greatly increased. Highly reactive nickel pow-

der is ultimately dropped through the outlet 20 into the hopper 21 filled with water, so that the hot nickel powder is cooled in the absence of air, thus minimizing objectionable oxidation of the nickel powder. Highly reactive nickel produced in this manner is most effectively employed in the cementation of copper and the neutralization of acidic nickel electrolyte.

I claim:—

- 5 1. The improvement in the method of preparing reactive metallic nickel powder by the reduction of nickel oxide, nickel-copper oxide and the like, which comprises progressively advancing the nickel oxide bearing material in finely divided form through a reduction zone in a direction generally countercurrent to and in direct contact with hot reducing gases, and at the same time indirectly heating the nickel oxide bearing material during its first stages of movement through the reduction zone, said hot reducing gases being introduced into the final stage of the reduction zone at a temperature between 500-700° C. to heat the material directly during its final stages of reduction and to main-

tain the treated material leaving the reduction zone at a temperature between 400-550° C. whereby sintering of the material is avoided and a highly reactive nickel powder is obtained.

- 10 2. The improvement in the method of preparing reactive metallic nickel powder by the reduction of nickel oxide, nickel-copper oxide and the like, which comprises progressively advancing the nickel oxide bearing material in finely divided form through a reduction zone in a direction generally countercurrent to and in direct contact with hot reducing gases, and at the same time indirectly heating the nickel oxide bearing material during its first stages of movement through the reduction zone, said hot reducing gases being introduced into the final stage of the reduction zone at a temperature sufficiently high to heat the material directly during its final stages of reduction and to maintain the treated material leaving the reduction zone at a 15 temperature between 400-550° C. whereby sintering of the material is avoided and a highly reactive nickel powder is obtained.

ANTON MARTIN GRONNINGSAETER.